

Patented Feb. 29, 1944

2,343,051

# UNITED STATES PATENT OFFICE

2,343,051

## PROCESS FOR PREPARING PHOTOGRAPHIC SILVER HALIDE EMULSIONS FOR MULTI-COLOR PHOTOGRAPHY

Alfred Fröhlich and Wilhelm Schneider, Dessau, and Gustav Wilmanns, Wolfen, Kreis Bitterfeld, Germany, assignors to General Aniline & Film Corporation, New York, N. Y., a corporation of Delaware

No Drawing. Application July 13, 1940, Serial No. 345,364. In Germany July 13, 1939

8 Claims. (Cl. 95—7)

The present invention relates to color photography and more particularly to an improved method of preparing photographic silver halide emulsions for multi-color photography.

It is known that color formers fast to diffusion are employed for the manufacture of photographic color images. These color formers fast to diffusion cannot be removed from the emulsion layer by the usual photographic treating baths, for instance by washing, though they have been added to the silver halide emulsion in dissolved form. As such color formers there were proposed for instance substances which are insoluble in aqueous alkalies, the hydrogen ion concentration of which corresponds approximately to that of the usual photographic developing solutions, which, however, are soluble at increased alkalinity, for instance in diluted caustic soda solution. These color formers are incorporated into the emulsion dissolved in diluted caustic soda solution. It is known furthermore to dissolve scarcely soluble components in organic solvents, for instance methanol partly with the aid of caustic alkalies and to add these solutions to the photographic emulsion, thereby accomplishing the necessary dispersion of the precipitated difficultly soluble substance in the solution by means of violent stirring or by means of precipitating or dispersing agents.

If there are employed color formers fast to diffusion which contain groups effecting better water solubility, such as acid- or hydroxyl groups, they may be dissolved in diluted soda solution, whereby these soda-alkaline solutions possess a pH-value which approximately corresponds to that of the photographic developing solution. This pH-value amounting to about 11, is, however, not very suitable for photographic emulsions, especially for sensitized emulsion layers, since the addition of the solution of the color former influences the pH-value. This causes nearly always an increase in sensitivity which, however, is entirely undesired at this moment, as the process is hard to control. Such highly sensitive emulsions, moreover, are inclined to fogging and possess low keeping quality.

The present invention has for an object to provide color components which are soluble in the emulsion layer and which are fast to diffusion with respect to the different photographic treating processes afterwards.

A further object is to provide silver halide emulsions containing the color forming components fast to diffusion.

A further object is to provide an improved film

for color photography having superposed silver halide emulsion layers, each layer containing a color component fast to diffusion.

These and other objects will become apparent from the following specification.

It has been found, that these difficulties can be avoided and that excellent stable emulsions for multi-color photography are obtained, if a pH-value of about 5-8 is chosen for the finished emulsion layers. For that purpose it is first of all necessary that the color formers fast to diffusion which are to be added to the emulsion are soluble at a pH-value of less than 9. To dissolve therefore these components an alkalinity must be sufficient which in no case is higher than pH=9. In order to accomplish the desired solubility with regard to color components fast to diffusion, the kind and number of the groups which effect improved water-solubility and which have to be introduced into the molecule, have to be chosen according to the kind and number of the molecule radicals which effect fastness to diffusion.

Such color formers fast to diffusion which possess molecule-radicals and acid groups incorporating fastness to diffusion or which have other substituents effecting soda- or water-solubility are for instance the following: 1-naphthol-2-carboyl - amino - phenyl-3'-octadecylamino-4'-sulfo acid- 4'-sulfo acid, 1 - naphthol-2-carboylamino-phenyl-3'-octadecylamino-4'-carboxylic acid - 4'-sulfo acid, 1-naphthol-2-carboylaminophenyl-3'-oleylamino-4'-sulfo acid-4'-sulfo acid, 1-naphthol-2-carboylaminophenyl-3'-dodecylamino-4'-sulfo acid-4'-sulfo acid, 1-naphthol-2-carboyl-aminophenyl-3'-abietylamino - 4' - sulfo acid-4'-sulfo acid, 1-naphthol-2-carboylaminophenyl-3'-cholylamino-4'-sulfo acid-4'-sulfo acid, 2-sulfo-oleylamino-1-naphthol-4'-sulfo acid, 1-naphthol-2-carboylaminocholesterin-4'-sulfo acid, 1-naphthol-2-carboylabietylamine-4'-sulfo acid, 1-naphthol-2-carboylamino-4'-sulfooleylphenyl- 4 - sulfo acid, 1-naphthol-2-carboylamino-4'-heptadecyl-aminobenzene-2'-sulfo acid-4'-sulfo acid, 1-naphthol-2-carboylamino-3'- sulfooleylaminobenzene-4'-sulfo acid, di-1,1'-naphthoxy-2,2'-carboyl-3'-stearylarnino - benzidine - 4,4' - sulfo acid, 1,2,3-xylenolcarboylactadecylamino - 4 - sulfo acid, 1-naphthol - 6 - sulfonylheptadecylamino - 4 - sulfo acid, 6 - methoxy-1-naphthol - 2 - carboyl-sulfo-oleylamino-4 - sulfo acid, 1-naphthol-2-carboyl-amino - 4'-methylhepta - decylaminobenzene-3'-sulfo acid-4'-sulfo acid, 1-naphthol-2-carboyl-amino-4'-methylsulfo - octadecylaminobenzene-4'-sulfo acid, 8-octadecylethylamino-1-naphthol-2,4-disulfo acid, mixture from  $\alpha$ -oxynaphthoic

acid and polyethyleneoxide, mixture from  $\alpha$ -oxy-naphthoic acid and aminophenylpolyethylene-oxideether, 4 - sulfooleylaminobenzoylacetylaminono - 3',4' - benzenedicarboxylic acid, laurylacetic acid aminebenzenedicarboxylic acid, 1-(3',6'-dimethyl-3'-stearoylaminoo) - phenyl-3-methyl-5-pyrazolone-4'-sulfo acid, 1,3'-carboxyphenyl - 3-4'-sulfooleylaminophenyl-5-pyrazolone, 1,5'-carboxy-3' - sulfooleylaminophenyl- 3 - furfuryl- 5 - pyrazolone, 1-phenyl- 3 - palmitoyl-5-pyrazolone-3',5'-disulfo acid, 1-phenyl-3-palmitoyl-5-pyrazolone-3'-sulfo acid - 4' - methylaminooethanesulfo acid, 1-phenyl- 3 - sulfoheptadecyl- 5 - pyrazolone, 1,3'-sulfooleylaminophenyl- 3 - methyl-5-pyrazolone, 1,3'-sulfooleylaminophenyl-5-pyrazolone-3-acetic acid, 5-pyrazolone-3-acetic acid-1-( $\beta$ -octadecyl- $\alpha$ -carboxylic acid).

Color formers fast to diffusion according to the below-mentioned U. S. patents are, generally speaking, very suitable, the solubility of which has been set by the introduction of groups effecting improved water solubility to a pH-value being smaller than 9: 2,178,612, of November 7, 1939; 2,179,238, of November 7, 1939; 2,179,244, of November 7, 1939; 2,186,732, of January 9, 1940; 2,186,849, of January 9, 1940; 2,186,850, of January 9, 1940; 2,280,722, of April 21, 1942; 2,307,399, January 5, 1943.

The components may also be dissolved at a stronger alkalinity than pH-value=9 and the solution may then be set at a pH-value of at least not more than 9 by adding diluted acid. Furthermore the solution of a color former having stronger alkalinity may be added to the emulsion during the manufacturing process or before casting and there may be added to the emulsion so much of a diluted acid or of an acid salt, as is necessary for the neutralization of the alkali which is not bound to the color former. Condition is, however, in all these cases, that the color formers are soluble at a pH-value of less than 9.

The emulsions naturally may contain all modifying agents suitable for the manufacture of photographic emulsions. With regard to the final

pH-value of the emulsion, also the effect of the modifying agents has to be taken into consideration.

We claim:

- 5 1. Process for the manufacture of silver halide emulsions for color photography, which process comprises dissolving in alkali, color components fast to diffusion in gelatin and completely soluble at a pH value of about 9, incorporating the alkaline color former solution into the emulsion at a pH of about 9, and reducing the alkalinity of the mixture by neutralizing to a pH value of from 5 to 8.
- 10 2. The process as defined in claim 1, wherein the color component is fast to diffusion by virtue of the presence therein of a long aliphatic chain.
- 15 3. The process as defined in claim 1, wherein the color component is fast to diffusion by virtue of the presence therein of a long aliphatic chain and wherein the color component contains a plurality of water-solubilizing groups.
- 20 4. The process as defined in claim 1, wherein the color component is fast to diffusion by virtue of the presence therein of a long aliphatic chain and wherein the color component contains a plurality of sulfonic acid groups.
- 25 5. The process as defined in claim 1, wherein the color component is a naphthol containing a long aliphatic chain.
- 30 6. The process as defined in claim 1, wherein the color component is a naphthol containing a long aliphatic chain and a plurality of water-solubilizing groups.
- 35 7. The process as defined in claim 1, wherein the color component is a pyrazolone containing a long aliphatic chain.
- 40 8. The process as defined in claim 1, wherein the color component is a pyrazolone containing a long aliphatic chain and a plurality of water-solubilizing groups.

ALFRED FRÖHLICH.  
WILHELM SCHNEIDER.  
GUSTAV WILMANNS.